

## UNITED STATES PATENT OFFICE

2,106,554

## LUBRICATING OILS

Bert H. Lincoln and Alfred Henriksen, Ponca City, Okla., assignors, by mesne assignments, to The Lubri-Zol Development Corporation, Cleveland, Ohio, a corporation of Delaware

No Drawing. Application June 22, 1932,  
Serial No. 618,704

10 Claims.

(Cl. 87-9)

Our invention relates to lubricating oils and more particularly to improved methods for the production of high quality lubricating oils and such products as new compositions of matter.

- 5 It is well known that mineral lubricating oils are deficient in oiliness characteristics, which is the most important character of the lubricant when used under conditions of boundary lubrication, where the viscosity of the lubricant plays 5  
10 little or no part in lubrication. Boundary lubrication conditions are obtained when engines are operating at heavy load, low speeds or, if for any reason, the supply of lubricant is cut off or not sufficient. This last condition may exist when 15  
15 for mechanical reasons the lubricant pump is not functioning properly or when the lubricant feed line is clogged with foreign matter.

It has been known that hydrocarbons of the aliphatic series, such as are found in petroleum oils 20 or distillates, and aromatic hydrocarbons having an aliphatic side chain attached to the nucleus, such as the hydrocarbons occurring in the products of the destructive distillation of coal or wood, may be oxidized under properly controlled 25 conditions of pressure and temperature by means of oxygen, air or other oxidizing agents, with or without the use of a catalytic agent, to produce economical yields of certain oxidation products. These products usually contain organic acids containing the carboxyl group and the hydroxy acids, that is, acids containing both the carboxyl group 30 and one or more hydroxyl groups, as well as esters, lactones, aldehydes, ketones, etc.

The oxidation process is carried on by treating 35 the hydrocarbon to be oxidized at an elevated temperature with an oxidizing gas under pressure. The temperatures and pressures vary depending upon the hydrocarbon being treated and upon the speed with which the reaction is to take 40 place, and whether or not a catalyst is used to promote the reaction. It is to be remembered that these oxidation processes are known to the art and are not to be considered part of our invention.

45 One object of our invention is to provide a lubricant of high oiliness character, low coefficient of friction, and one which will act as a safety factor in lubrication when abnormal conditions exist for one reason or another.

50 Another object of our invention is to provide a lubricant which will maintain a very low coefficient of friction when diluted with light hydrocarbons such as are obtained in an automobile crank case by incomplete combustion of the fuel.

A further object of our invention is to provide a lubricant having penetrative lubricity characteristics. It has been found that our lubricant does not drain off the rubbing surfaces when idle, thereby providing a lubricating film on the rubbing surfaces at all times and being of great value to the life of the machine in cold weather starting when the lubricant is very viscous and sluggish.

5 It has been demonstrated a number of times 10 that hydrocarbon lubricants of the very best quality are not constant in coefficient of friction with slightly changing loads or speeds, and in some cases the coefficient of friction varies over rather wide limits with some lubricants when all 15 operating conditions are held constant.

Another object of our invention is to provide a lubricant which shows a more nearly constant coefficient of friction, thereby insuring smoother 20 engine operation.

In practicing our invention only small quantities of the various products are added to hydrocarbon lubricants. The product is well blended with the hydrocarbon and the mixture is ready for use. To prove the efficiency and value of our 25 invention, we determine the coefficient of friction of the original hydrocarbon lubricant by testing on the Herschel friction testing machine, which was developed by Dr. W. H. Herschel of the United States Bureau of Standards and is well 30 known to the art. The coefficient of friction of the mixture of hydrocarbon oil and oxidation product is then determined by the same machine.

We have further found that original hydrocarbon 35 lubricants and hydrocarbon lubricants blended with products have low film strength and have a tendency to break down and allow seizure of metals at relatively low pressures. The film strength of a lubricant is of great importance 40 when the lubricant is used under heavy loads and slow speeds. By halogenating the products of this invention prior to blending with hydrocarbon lubricants the film strength is greatly improved.

In general, our invention contemplates the addition of small quantities of oxidation products of hydrocarbons to a petroleum hydrocarbon oil to increase the lubricity of the oil. Due to the fact that the film strength of the hydrocarbon 50 oil, with which a small percentage of hydrocarbon oxidation products is added, is low, we halogenate the oxidation products before their addition, in order to increase the film strength, as will be hereinafter fully described.

More particularly, the following example of one method of carrying out our invention is given. It is to be understood, however, that this example is not to be considered a limitation of our invention, but is merely given by way of illustration to enable those skilled in the art to practice our invention.

We oxidize hydrocarbons and wax to form acids and esters by any of the methods shown in the following patents: Burwell, 1,690,769; Mackenzie et al., 1,705,298; Pungs et al., 1,787,951; McCoull, 1,767,147; Burwell, 1,690,768. The oxidation product thus obtained, as for example according to the Burwell process, in which a petroleum hydrocarbon oil is oxidized in the presence of a manganese compound in the neighborhood of 120° C. under about 300 pounds' pressure, is then treated with chlorine at room temperature. Excess chlorine and hydrogen chloride are removed by warming and washing with solvents. The product thus prepared was then added to a sample of high quality lubricant and tested on the Timken machine, which is a machine for determining film strength of lubricants, developed and manufactured by the Timken Roller Bearing Company and well known in the art. A sample of the original hydrocarbon lubricant was also tested on the Timken machine. Likewise the hydrocarbon lubricant with the addition of the aforescribed oxidation product was tested on the Timken machine. The following results were obtained:

| 35 | Product                                                                             | Pound weight reading | Film strength lbs./sq. inch |
|----|-------------------------------------------------------------------------------------|----------------------|-----------------------------|
|    | Original hydrocarbon.....                                                           | 18.2                 | 10,500                      |
| 40 | Original hydrocarbon plus $\frac{1}{4}$ of 1% of oxidation product.....             | 20.7                 | 12,000                      |
|    | Original hydrocarbon plus $\frac{1}{4}$ of 1% of chlorinated oxidation product..... | 35.2                 | 20,000                      |

It will be obvious from the foregoing that the film strength obtained by the addition of a small quantity of a chlorinated oxidation product will practically double the film strength.

The oxidation product appears to be a mixture of acids, hydroxy acids, esters, lactones, etc., of rather indefinite and widely varying composition. This, however, is unimportant inasmuch as it is efficient and produces the results upon which the invention is based. Varying quantities of chlorinated product may be added depending upon the quality of the initial lubricant. As a general rule, we have found that quantities varying from 0.1% to 2% are sufficient for normal lubricants of salable quality. We have found that a limiting percentage is usually reached, after which the film strength does increase for the particular lubricating oil with which the halogenated oxidation product is added. In some cases it may be necessary to add as much as 5%, if the lubricant is of a very poor quality, to obtain a marked increase in the film strength.

65 A mineral oil which had a coefficient of friction of .140 as tested on the Herschel machine was again tested after the addition of a small percentage of the oxidation product of a hydrocarbon oil obtained as described above. The resulting coefficient of friction was .075, clearly showing a marked increase in the lubricating quality of the oil.

It will be understood that certain features and sub-combinations are of utility and may be employed without reference to other features and sub-combinations. This is contemplated by and is within the scope of our claims. It is further obvious that various changes may be made in details within the scope of our claims without departing from the spirit of our invention. It is, therefore, to be understood that our invention is not to be limited to the specific details shown and 10 described.

Having thus described our invention, what we claim is:

1. A lubricating oil comprising in combination, a major quantity of a hydrocarbon oil and a minor quantity of the halogenated oxygeniferous product obtained by chlorinating the immediate product obtained by oxidizing a hydrocarbon. 15

2. A lubricating oil comprising in combination, a hydrocarbon oil and a small quantity of the halogenated oxygeniferous product obtained by chlorinating the immediate product obtained by subjecting a hydrocarbon to the action of oxygen under heat and pressure. 20

3. A lubricating oil comprising in combination a major quantity of a hydrocarbon oil and a minor quantity of a halogenated, oxygeniferous product obtained by chlorinating the immediate product obtained by oxidizing an aliphatic hydrocarbon. 25

4. A lubricating oil comprising in combination a major quantity of a hydrocarbon oil and a minor quantity of the halogenated oxygeniferous product obtained by halogenating the immediate product obtained by oxidizing a hydrocarbon. 30

5. A lubricating oil comprising in combination a major quantity of a hydrocarbon oil and a minor quantity of a halogenated, oxygeniferous product obtained by halogenating the immediate product obtained by oxidizing an aliphatic hydrocarbon. 35

6. A lubricating oil comprising in combination a major quantity of a hydrocarbon oil and a minor quantity of the halogenated oxygeniferous products obtained by halogenating the immediate product obtained by oxidizing a complex mixture of hydrocarbons. 40

7. A lubricating oil comprising in combination a major quantity of a hydrocarbon oil and a minor quantity of the halogenated oxygeniferous products obtained by halogenating the immediate product of oxidation of a hydrocarbon wax. 45

8. A lubricating oil comprising in combination a major quantity of a hydrocarbon oil and from 0.1% to 5% of an oxygen and halogen bearing product of the type obtained by the oxidation of hydrocarbons and the halogenation of the hydrocarbons thus oxidized. 55

9. A lubricating oil comprising in combination a major quantity of a hydrocarbon oil and from 0.1% to 2% of an oxygen- and halogen-bearing product of the type obtained by the oxidation of hydrocarbons and the halogenation of the hydrocarbons thus oxidized. 60

10. A lubricating oil comprising in combination a major quantity of a hydrocarbon oil and from 0.1% to 5% of an oxygen- and chlorine-bearing product of the type obtained by the oxidation of hydrocarbons and the chlorination of the hydrocarbons thus oxidized. 65

BERT H. LINCOLN.  
ALFRED HENRIKSEN.